



US005866309A

# United States Patent [19]

Fitterman et al.

[11] Patent Number: 5,866,309

[45] Date of Patent: Feb. 2, 1999

[54] **METHOD FOR PROCESSING ROOMLIGHT HANDLEABLE PHOTOGRAPHIC ELEMENTS**

[76] Inventors: **Alan S. Fitterman; Jeffrey S. Baugher; Robert E. Dickerson**, all of Eastman Kodak Company, 343 State St., Rochester, N.Y. 14650

[21] Appl. No.: 956,305

[22] Filed: Oct. 22, 1997

[51] Int. Cl.<sup>6</sup> ..... G03C 5/29

[52] U.S. Cl. ..... 430/440; 430/446; 430/455; 430/963; 430/966

[58] Field of Search ..... 430/440, 446, 430/455, 963, 966

## [56] References Cited

### U.S. PATENT DOCUMENTS

|           |         |                  |       |         |
|-----------|---------|------------------|-------|---------|
| 2,688,549 | 9/1954  | James et al.     | ..... | 430/480 |
| 3,630,744 | 12/1971 | Thiers et al.    | ..... | 430/602 |
| 4,029,510 | 6/1977  | Speers           | ..... | 430/465 |
| 4,803,150 | 2/1989  | Dickerson et al. | ..... | 430/502 |
| 5,236,816 | 8/1993  | Purol et al      | ..... | 430/492 |
| 5,278,035 | 1/1994  | Knapp            | ..... | 430/452 |
| 5,370,977 | 12/1994 | Zietlow          | ..... | 430/502 |
| 5,376,510 | 12/1994 | Parker et al.    | ..... | 430/466 |

|           |        |                   |       |         |
|-----------|--------|-------------------|-------|---------|
| 5,384,232 | 1/1995 | Bishop et al.     | ..... | 430/440 |
| 5,389,502 | 2/1995 | Fitterman et al.  | ..... | 430/491 |
| 5,424,176 | 6/1995 | Schmittori et al. | ..... | 430/455 |
| 5,498,511 | 3/1996 | Yamashita et al.  | ..... | 430/496 |
| 5,652,086 | 7/1997 | Brayer et al.     | ..... | 430/398 |

### FOREIGN PATENT DOCUMENTS

|              |        |                    |   |
|--------------|--------|--------------------|---|
| 0 573 700 A1 | 6/1992 | European Pat. Off. | . |
| 0 585 792 A2 | 9/1992 | European Pat. Off. | . |
| 0 588 408 A1 | 8/1993 | European Pat. Off. | . |
| 95/00881     | 6/1993 | WIPO               | . |

Primary Examiner—Hoa Van Le  
Attorney, Agent, or Firm—J. Lanny Tucker

## [57] ABSTRACT

Black-and-white elements, such as radiographic films, can be handled and processed in roomlight because they include certain light absorbing dyes and desensitizers. Processing is carried out by developing the exposed element using a developing composition having a pH of less than 10. The developed elements are fixed using a fixing composition having a pH of from 10 to 11.5, and comprising specific amounts of fixing agent and sulfite to solubilize silver halide and to bleach or decompose the light absorbing dyes. The processing method is carried out quickly, usually within 120 seconds.

20 Claims, No Drawings

## METHOD FOR PROCESSING ROOMLIGHT HANDLEABLE PHOTOGRAPHIC ELEMENTS

### FIELD OF THE INVENTION

This invention relates in general to photography and in particular to an improved method for processing roomlight handleable, black-and-white photographic elements. More particularly, it relates to a method of processing roomlight handleable black-and-white radiographic films using specific developing and fixing solutions.

### BACKGROUND OF THE INVENTION

Roentgen discovered X-radiation by the inadvertent exposure of a silver halide photographic element. In 1913, Eastman Kodak Company introduced its first product specifically intended to be exposed by X-radiation (X-rays). Silver halide radiographic films account for the overwhelming majority of medical diagnostic images. It was recognized almost immediately that the high energy ionizing X-rays are potentially harmful, and ways were sought to avoid high levels of patient exposure. Radiographic films provide viewable silver images upon imagewise exposure followed by rapid access processing.

One approach, still in wide-spread use is to coat the silver halide emulsions useful in radiographic films on both sides of the film support. Thus, the number of X-rays that can be absorbed and used for imaging are doubled, providing higher sensitivity. Dual-coated radiographic films are sold by Eastman Kodak Company under the trademark DUPLITIZED films. Films that rely entirely on X-radiation absorption for image capture are referred to in the art as "direct" radiographic elements, while those that rely on intensifying screen light emission are referred to as "indirect" radiographic elements. Because the silver halide emulsions are used to capture the X-rays directly in "direct" films, the coating coverages of such emulsions are generally higher than in other radiographic elements. A typical coverage is about 5 g of silver/m<sup>2</sup> per side of DUPLITIZED films, and twice that amount for single-side coated films.

Other radiographic films are considered "indirect" because they are used in combination with phosphor-containing X-ray intensifying screens that absorb the X-rays, and then emit light that exposes the silver halide grains in the emulsion layers.

In addition to the two broad categories noted above, there is a third category of radiographic films, most commonly used for dental intra-oral diagnostic imaging and hereafter referred to as dental films. Intra-oral dental imaging presents obvious barriers to the use of intensifying screens. Thus, dental films utilize the coated silver halide to absorb X-rays, and are therefore a form of "direct" radiographic films.

There are other applications for direct radiographic films, such as in various industrial applications where X-rays are captured in imaging, but intensifying screens cannot be used for some reason.

U.S. Pat. No. 5,370,977 (Zietlow) describes dental films having improved characteristics and containing certain tabular grain silver halide emulsions. No spectral sensitization is used in such dental films, but in order to avoid fogging the films with inadvertent light exposure, the emulsions contain what is identified as a "desensitizer" that reduces emulsion sensitivity to light. Conventional processing solutions and conditions are described for these dental films.

Other desensitizing compounds for radiographic films are described in U.S. Pat. No. 3,630,744 (Thiers et al) for

reducing film sensitivity to roomlight and UV radiation. Conventional processing of these films is also described.

Double-coated indirect radiographic elements described in U.S. Pat. No. 4,803,150 (Dickerson et al) contain certain microcrystalline particulate dyes that reduce "crossover". These elements are designed for use with intensifying screens. Crossover occurs when some light emitted by the screen passes through the film support and exposes silver halide grains on the opposite side, resulting in reduced image sharpness. The noted particulate dyes absorb unwanted crossover exposure, but can be decolorized during conventional processing. Thus, a pH 10 developing solution is described for its conventional use as well as to decolorize the dyes within 90 seconds. Conventional fixing and washing follow.

It is the prevailing practice to process direct radiographic films for 3 or more minutes because of the higher silver coating coverages. Such processes typically include black-and-white development, fixing, washing and drying. Films processed in this manner are then ready for image viewing.

Photographic developing solutions containing a silver halide developing agent are well known in the photographic art for reducing silver halide grains containing a latent image to yield a developed photographic image. Many useful developing agents are known in the art, with hydroquinone and similar dihydroxybenzene compounds and ascorbic acid (and derivatives) being some of the most common. Such solutions generally contain other components such as sulfites, buffers, antifoggants, halides and hardeners. A workable pH for such solution is usually in the range of from about 10 to about 11, depending upon the developing agent and other solution components.

Fixing solutions for radiographic films are also well known and include one or more fixing agents, of which thiosulfates are most common. Such solutions generally include sulfites as antioxidants, and hardeners, and have a functional pH range of from about 4 to about 5.5.

Direct radiographic films, including dental films, thus have some sensitivity to roomlight and UV as well as X-rays, and therefore care must be taken to avoid inadvertent room-light exposure before and during processing. There has been a desire for radiographic films that are less sensitive to roomlight, and that can be handled and processed without the need for a darkroom or other special conditions. Such films would have a number of useful applications, such as dental and industrial imaging. However, conventional processing solutions and methods cannot be used to provide suitable radiographic images in such films.

### SUMMARY OF THE INVENTION

The present invention provides an advance in the art with a method for providing a black-and-white image comprising:

- 55 A) contacting an imagewise exposed photographic silver halide element with an aqueous black-and-white developing composition having a pH of less than 10, and
- 60 B) contacting the element with a fixing composition having a pH of from 10 to 11.5, and comprising a fixing agent at from about 0.8 to about 2.5 mol/l and a sulfite at from about 0.1 to about 0.3 mol/l, wherein steps A and B require a total of from about 40 to about 120 seconds, and the element comprising a support having thereon one or more layers, at least one of the layers being a silver halide emulsion layer, the element further comprising:

in one of the layers, a microcrystalline particulate dye that absorbs electromagnetic radiation in the visible and UV portions of the spectrum and is decolorized during step B, and

in each silver halide emulsion layer, a desensitizer that reduces sensitivity of the silver halide emulsion layer to electromagnetic radiation in the visible portion of the spectrum by trapping electrons generated by exposure to that electromagnetic radiation.

The present invention provides a means for processing radiographic elements in roomlight. Such films and processing would find considerable advantage for dental applications as well and some industrial uses. Thus, a conventional darkroom is unnecessary. In preferred embodiments, the elements are direct radiographic films having a silver halide emulsion layer on both sides of the film support.

These advantages are achieved by a unique combination of element composition and processing compositions and conditions. First of all, the processed element contains a particulate dye that absorbs visible and UV radiation, but not to X-rays. These dyes enable roomlight handleability, but they are then decolorized during processing, particularly during fixing. In addition, further light protection is provided in the element by the presence of a silver halide desensitizer to trap electrons released by photo-exposure, but which dyes obviously are not affected by X-rays.

The processing compositions and conditions used in the invention are designed to decolorize the particulate dye after development while providing rapid image formation. Thus, the developing solution must have a lower pH than is conventional, that is below 10. The developing agent must then be chosen to be soluble at that lower pH, and in most cases, the dihydroxybenzene compounds are not suitable, but ascorbic acid developing agents are more generally useful at the lower pH. It is critical that the pH of the developing composition be lower than the fixing solution so the particulate dye is decolorized during fixing not development. Conventional fixing solutions have a pH below 6, but in the present invention, it is from 10 to about 11.5 in order to accommodate high amounts of sulfite that decolorizes or deactivates the particulate dye.

In preferred embodiments, an acidic final washing solution is used after fixing to stop further development and to remove fixing agent.

#### DETAILED DESCRIPTION OF THE INVENTION

The present invention is useful for providing a black-and-white image in a photographic silver halide element, and preferably a radiographic film. Other elements that can be processed using the present invention include, but are not limited to, aerial films, black-and-white motion picture films, duplicating and copy films, and amateur and professional continuous tone black-and-white films. The components of such materials are well known in the art but the specific features that make them roomlight handleable are described below in more detail.

The aqueous black-and-white developing composition useful in the practice of this invention contains one or more black-and-white developing agents, including dihydroxybenzene and derivatives thereof, and ascorbic acid and derivatives thereof. Preferably, the composition is free of dihydroxybenzene and its derivatives because such developing agents are usually not suitably soluble at pH below 10. The concentration of sulfite in the developing solution is generally lower than that found in conventional developing solutions, especially when it is free of dihydroxybenzene

developing agents. Because of the lower levels of sulfite and lower pH of the developing composition, the particulate dyes (described below) are not decolorized until the fixing step.

Ascorbic acid developing agents are described in a considerable number of publications in photographic processes, including U.S. Pat. No. 5,236,816 (Purol et al) and references cited therein. Useful ascorbic acid developing agents include ascorbic acid and the analogues, isomers and derivatives thereof. Such compounds include, but are not limited to, D- or L-ascorbic acid, sugar-type derivatives thereof (such as sorboascorbic acid, g-lactoascorbic acid, 6-desoxy-L-ascorbic acid, L-ramnoascorbic acid, imino-6-desoxy-L-ascorbic acid, glucoascorbic acid, fucoascorbic acid, glucoheptoascorbic acid, maltoascorbic acid, L-arabosascorbic acid), sodium ascorbate, potassium ascorbate, isoascorbic acid (or L-erythroascorbic acid), and salts thereof (such as alkali metal, ammonium or others known in the art), endiol type ascorbic acid, an enaminol type ascorbic acid, a thiolenol type ascorbic acid, and an enamin-thiol type ascorbic acid, as described for example in U.S. Pat. No. 5,498,511 (Yamashita et al), EP-A-0 585,792 (published Mar. 9, 1994), EP-A-0 573 700 (published Dec. 15, 1993), EP-A-0 588 408 (published Mar. 23, 1994), WO 95/00881 (published Jan. 5, 1995), U.S. Pat. No. 5,089,819 and U.S. Pat. No. 5,278,035 (both of Knapp), U.S. Pat. No. 5,384,232 (Bishop et al), U.S. Pat. No. 5,376,510 (Parker et al), Japanese Kokai 7-56286 (published March 3, 1995), U.S. Pat. No. 2,688,549 (James et al), U.S. Pat. No. 5,236,816 (noted above) and *Research Disclosure*, publication 37152, March 1995. D-, L-, or D,L-ascorbic acid (and alkali metal salts thereof) or isoascorbic acid (or alkali metal salts thereof) are preferred. Sodium ascorbate and sodium isoascorbate are most preferred. Mixtures of these developing agents can be used if desired.

The developing composition can also include one or more auxiliary co-developing agents, which are also well known (e.g., Mason, *Photographic Processing Chemistry*, Focal Press, London, 1975).

Any auxiliary developing agent can be used, but the 3-pyrazolidone developing agents are preferred (also known as "phenidone" type developing agents). Such compounds are described, for example, in U.S. Pat. No. 5,236,816 (noted above). The most commonly used compounds of this class are 1-phenyl-3-pyrazolidone, 1-phenyl-4,4-dimethyl-3-pyrazolidone, 4-hydroxymethyl-4-methyl-1-phenyl-3-pyrazolidone, 5-phenyl-3-pyrazolidone, 1-p-aminophenyl-4,4-dimethyl-3-pyrazolidone, 1-p-tolyl-4,4-dimethyl-3-pyrazolidone, 1-p-tolyl-4-hydroxymethyl-4-methyl-3-pyrazolidone, and 1-phenyl-4,4-dihydroxymethyl-3-pyrazolidone. Other useful co-developing agents comprise one or more solubilizing groups, such as sulfo, carboxy or hydroxy groups attached to aliphatic chains or aromatic rings, and preferably attached to the hydroxymethyl function of a pyrazolidone, as described for example, in commonly assigned and copending U.S. Ser. No. 08/694,792 filed Aug. 9, 1996, by Roussille et al. A most preferred co-developing agent is 4-hydroxymethyl-4-methyl-1-phenyl-3-pyrazolidone.

Less preferred auxiliary co-developing agents include 60 aminophenols such as p-aminophenol, o-aminophenol, N-methylaminophenol, 2,4-diaminophenol hydrochloride, N-(4-hydroxyphenyl)glycine, p-benzylaminophenol hydrochloride, 2,4-diamino-6-methylphenol, 2,4-diaminoresorcinol and N-(beta-hydroxyethyl)-p-aminophenol.

A mixture of different types of auxiliary developing agents can also be used if desired.

Various organic antifoggants can be used in the developing solution, either singly or in admixture. Such compounds control the gross fog appearance in the processed elements. Suitable antifoggants include, but are not limited to, benzimidazoles, benzotriazoles, mercaptotetrazoles, indazoles and mercaptothiadiazoles. Representative antifoggants include 5-nitroindazole, 5-p-nitrobenzoylaminoimidazole, 1-methyl-5-nitroindazole, 6-nitroindazole, 3-methyl-5-nitroindazole, 5-nitrobenzimidazole, 2-isopropyl-5-nitrobenzimidazole, 5-nitrobenzotriazole, sodium 4-(2-mercapto-1,3,4-thiadiazol-2-yl-thio)butanesulfonate, 5-amino-1,3,4-thiadiazol-2-thiol, 5-methylbenzotriazole, benzotriazole and 1-phenyl-5-mercaptotetrazole. Benzotriazole is most preferred.

The developing composition also includes one or more preservatives or antioxidants. Various conventional black-and-white preservatives can be used including sulfites. A "sulfite" preservative is used herein to mean any sulfur compound that is capable of forming or providing sulfite ions in aqueous alkaline solution. Examples include, but are not limited to, alkali metal sulfites, alkali metal bisulfites, alkali metal metabisulfites, amine sulfur dioxide complexes, sulfuric acid and carbonyl-bisulfite adducts. Mixtures of these materials can also be used.

Examples of preferred sulfites include sodium sulfite, potassium sulfite, lithium sulfite, sodium bisulfite, potassium bisulfite, sodium metabisulfite, potassium metabisulfite and lithium metabisulfite. The carbonyl-bisulfite adducts that are useful include alkali metal or amine bisulfite adducts of aldehydes and bisulfite adducts of ketones. Examples of these compounds include sodium formaldehyde bisulfite, sodium acetaldehyde bisulfite, succinaldehyde bis-sodium bisulfite, sodium acetone bisulfite, b-methyl glutaraldehyde bis-sodium bisulfite, sodium butanone bisulfite, and 2,4-pentandione bis-sodium bisulfite.

Various known buffers can be included in the solutions to maintain the desired pH below 10. Carbonate is preferred in the practice of this invention. The pH of the developing solution is preferably less than 9.5 and more preferably less than 9. The pH is generally greater than 7 and more preferably greater than 8.

It is also optional that the developing compositions described herein contain one or more sequestering agents that typically function to form stable complexes with free metal ions (such as silver ions) in solution. Many useful sequestering agents are known in the art, but particularly useful classes of compounds include, but are not limited to, multimeric carboxylic acids as described in U.S. Pat. No. 5,389,502 (Fitterman et al), aminopolycarboxylic acids, polyphosphate ligands, ketocarboxylic acids, and alkanolamines. Representative sequestering agents include ethylenediaminetetraacetic acid, diethylenetriaminepentaacetic acid, 1,3-propylenediaminetetraacetic acid, 1,3-diamino-2-propanoltetraacetic acid, ethylenediaminodisuccinic acid and ethylenediaminomonosuccinic acid.

The developing composition can contain other additives including various development restrainers, development accelerators, swelling control agents and stabilizing agents, each in conventional amounts. Examples of such optional components are described in U.S. Pat. No. 5,236,816 (noted above), U.S. Pat. No. 5,474,879 (Fitterman et al), Japanese Kokai 7-56286 and EP-A-0 585 792.

The essential components described above are present in the aqueous developing composition in the general and preferred amounts listed in Table I, all minimum and maximum amounts being approximate (that is, "about"). If for-

mulated in dry form, the developing solutions would have the essential components in amounts readily apparent to one skilled in the art suitable to provide the liquid concentrations.

TABLE I

| Component                      | General Amount    | Preferred Amount  |
|--------------------------------|-------------------|-------------------|
| Ascorbic acid developing agent | 110 to 220 mmol/l | 150 to 200 mmol/l |
| Co-developing agent            | 10 to 30 mmol/l   | 15 to 25 mmol/l   |
| Antifoggant                    | 10 to 25 mmol/l   | 13 to 21 mmol/l   |
| Sulfite antioxidant            | 125 to 300 mmol/l | 200 to 280 mmol/l |

All compositions useful in the method of this invention are prepared by dissolving the components in water and adjusting the pH to the desired value using acids or buffers. The compositions can also be provided in concentrated form, and diluted to working strength just before use, or during use. The components of the compositions can also be provided in a kit of two or more parts to be combined and diluted with water to the desired strength and placed in the processing equipment. The compositions can be used as their own replenisher, or another similar solution can be used as the replenishers.

Processing can be carried out in any suitable processor for a given type of photographic element. For example, for radiographic films, the method can be carried out using the processor described in U.S. Pat. No. 3,545,971 (Barnes et al). One suitable processor is sold by Eastman Kodak Company under the trademark X-OMAT.

In most instances, the processed element is a film sheet, but it can also be a continuous element. Each element is bathed in a processing composition for a suitable period of time.

The fixing composition useful in this invention contains one or more fixing agents, such as thiosulfates (including sodium thiosulfate, ammonium thiosulfate, potassium thiosulfate and others readily known in the art), mercaptot-substituted compounds (such as those described by Haist, *Modern Photographic Processing*, John Wiley & Sons, New York, 1979), thiocyanates (such as sodium thiocyanate, potassium thiocyanate, ammonium thiocyanate and other readily known in the art), amines, halides or sulfites. Mixtures of fixing agents can be used if desired. In a preferred embodiment, a mixture of a thiocyanate (such as sodium thiocyanate) and a thiosulfate (such as sodium thiosulfate) is used. In such mixtures, the molar ratio of a thiosulfate to a thiocyanate is from about 2:1 to about 1:3, and preferably from about 1:1 to about 1:2. The sodium salt fixing agents are preferred for environmental advantages.

The fixing composition also includes a sulfite in an amount sufficient to decolorize or deactivate the particulate dye(s) present in the processed photographic element. Any suitable sulfite, or mixture thereof, can be used, including but not limited to, those described above as useful in the developing composition.

The fixing composition can optionally include other addenda commonly used in fixing solutions, such as sequestering agents, fixing accelerators and buffers. The pH is critically higher than the pH of the developing composition, and is thus generally 10 or above, and less than about 11.5. Preferably, the pH is at least 10.4, and more preferably, at least 10.5. Preferably, the pH is less than 11, and more preferably less than 10.8. The pH can be provided by adding a suitable buffer, chemical base, or from the amount of

sulfite in the solution. Because of the higher fixing pH, hardening agents commonly used to reduce element swelling, are generally not present.

The useful and preferred amounts of fixing composition components are shown in the following Table II with the minimum and maximum amounts being approximate (that is, "about"):

TABLE II

| COMPONENT          | GENERAL AMOUNT   | PREFERRED AMOUNT   |
|--------------------|------------------|--------------------|
| Fixing agent(s)    | 0.8 to 2.5 mol/l | 1 to 2.25 mol/l    |
| Sulfite            | 0.1 to 0.3 mol/l | 0.15 to 0.25 mol/l |
| Sequestering agent | 2 to 5 mmol/l    | 3 to 4 mmol/l      |

Fixing is preferably, but not essentially, followed by a suitable washing step to remove silver salts dissolved by fixing and excess fixing agents, and to reduce swelling in the element. The wash solution can be water, but preferably the wash solution is acidic, and more preferably, the pH is 7 or less, and preferably from about 4.5 to about 7, as provided by a suitable chemical acid or buffer.

After washing, the processed elements may be dried for suitable times and temperatures, but in some instances the black-and-white image may be viewed in a wet condition.

Processing times and conditions for the invention are listed in the following Table III with the minimum and maximum values being approximate (that is, "about"). The total time for development and fixing is at least 40 seconds, and preferably at least 60 seconds. Preferably, each of these steps is carried out within from about 15 to about 30 seconds. The total time for the entire processing method can be as high as 120 seconds, and preferably, as high as 90 seconds.

TABLE III

| PROCESSING STEP | TEMPERATURE (°C.) | TIME (sec) |
|-----------------|-------------------|------------|
| Development     | 15-30             | 20-60      |
| Fixing          | 15-30             | 20-60      |
| Washing         | 15-30             | 20-60      |

The elements processed using the present invention are composed of a conventional flexible, transparent film support (polyester, cellulose acetate or polycarbonate) that has applied to each side one or more photographic silver halide emulsion layers. For radiographic films, it is conventional to use blue-tinted support materials to contribute to the blue-black image tone sought in fully processed films. Polyethylene terephthalate and polyethylene naphthalate are preferred film supports.

In general, such elements, emulsions, and layer compositions are described in many publications, including *Research Disclosure*, publication 36544, September, 1994. *Research Disclosure* is a publication of Kenneth Mason Publications, Ltd., Dudley House, 12 North Street, Emsworth, Hampshire PO10 7DQ England.

Preferred silver halide emulsions include silver bromide and silver bromoiodide (having up to 15 mol % silver iodide). Preferred silver halide emulsions include forehardened tabular grain emulsions as described, for example, in U.S. Pat. No. 4,414,304 (Dickenson et al). These emulsions typically have thin tabular grains of predominantly silver bromide and up to 15 mol % silver iodide, an average thickness of less than about 0.3  $\mu\text{m}$ , and preferably, up to 3 mol % silver iodide and an average thickness of less than

about 0.2  $\mu\text{m}$ . The grains are usually dispersed in forehardened colloids, such as forehardened gelatin (using a conventional hardener). The emulsions also contain conventional addenda for providing desired coating and sensitometric properties, including but not limited to, sensitizing dyes, infrared opacifying dyes, stabilizers, antifoggants, antikinking agents, surfactants, latent-image stabilizers and other materials known in the art.

In some embodiments, the radiographic films processed according to this invention can also include a thiaalkylene bis(quaternary ammonium) salt in at least one layer, to increase imaging speed by acting as development accelerators. Such elements are described in more detail in U.S. Pat. No. 5,652,086 (Brayer et al) incorporated herein by reference.

The silver halide emulsion and other layers in the elements contain conventional hydrophilic colloid vehicles (with or without peptizers or other binders), typically gelatin or gelatin derivatives. Various synthetic polymer peptizers or binders can also be used alone or in combination with gelatin or gelatin derivatives.

Each element has one or more silver halide emulsion layers on each side of the support, and the layers on each or different sides can have the same or different compositions. Thus, the silver halides in the layers can be the same or different. In one embodiment, the radiographic films have two silver halide emulsion layers on both sides of the support, with the layers closest the support containing solely silver bromide grains. The silver coverages on each or both sides of the support can be the same or different. Generally, the total silver coverage on each side is at least about 5 g Ag/m<sup>2</sup>, and preferably at least about 15 g Ag/m<sup>2</sup>.

Each side of the element can also include a protective overcoat, or only one side can have an overcoat layer, such as a layer containing a hydrophilic colloid material and optionally any other addenda commonly (such as matting agents) used to modify the surface characteristics. The coating coverage of such layers is generally at least 0.6 g/m<sup>2</sup> of protective colloid, such as a gelatin. Conventional subbing layers can also be included to adhere the silver halide emulsion layers to the support. Other layers, such as interlayers, may be present in the element for conventional purposes, such as providing adhesion. Preferred elements contain an overcoat layer on at least one side of the support.

The total thickness of the coated layers on either or both sides of the elements can be at least 3  $\mu\text{m}$ , and preferably at least 4  $\mu\text{m}$ . The thickness is generally less than 7  $\mu\text{m}$ , and preferably less than 6  $\mu\text{m}$ .

As noted above, the elements processed using this invention contain one or more particulate dyes and/or one or more desensitizers to provide roomlight handleability. Such materials are thus useful if they absorb all incident electromagnetic radiation at from about 350 to about 700 nm.

Advantageously, the elements contain one or more particulate dyes are described above that absorb electromagnetic radiation in the visible and UV regions of the spectrum. These dyes are usually placed in the overcoat layer(s), but they can be in more than one location as long as they are readily decomposed during fixing.

Such particulate dyes generally have a size to facilitate coating and rapid decolorization during processing. In general, the smaller particles are best for these purposes, that is those having a mean diameter of less than 10  $\mu\text{m}$ , and preferably less than 1  $\mu\text{m}$ . The particulate dyes are most conveniently formed by crystallization from solution in sizes ranging down to 0.01  $\mu\text{m}$  or less. Conventional techniques

can be used to prepare dyes of the desired size, including ball milling, roller milling and sand milling.

An important criterion is that such dyes remain in particulate form in hydrophilic colloid layers of photographic elements. Various hydrophilic colloids can be used, as would be appreciated by a skilled worker in the art, including those mentioned herein for various layers. Where the particulate dyes are placed in overcoat layers, the particulate dyes are generally the only component besides the binder material.

Classes of useful particulate dyes include, but are not limited to, nonionic classes of compounds such as nonionic polymethine dyes, which include the merocyanine, oxonol, hemioxonol, styryl and arylidene dyes. Anionic dyes of the cyanine class may also be useful as long as they have the desired coatability properties (soluble at pH 5 to 6 and 40° C.) and remain in particulate form after coating. Some useful particulate dyes are described, for example, in U.S. Pat. No. 4,803,150 (Dickerson et al), incorporated herein by reference.

The useful amount of particulate dye in the elements is at least 0.5 g/m<sup>2</sup> on each side of the support, and preferably at least 0.7 g/m<sup>2</sup>. Generally, the upper limit of such materials is 2 g/m<sup>2</sup>, and preferably, less than 1.5 g/m<sup>2</sup> is used. Mixtures of particulate dyes can be used in one or more layers of the element.

The elements processed according to this invention also include one or more "desensitizers" in a silver halide emulsion layer(s) in order to provide additional visible and UV light protection. Conventional desensitizers can be used, as are known in photography and radiography. Various desensitizers are described, for example, in *Research Disclosure*, Vol. 308, December, 1989, publication 308119, Section III, the disclosure of which is incorporated herein by reference. Classes of such compounds include azomethine dyes (such as those described in U.S. Pat. No. 3,630,744 of Thiers et al).

Generally, the amount of desensitizer relative to the amount of silver halide in the element is adapted according to the particular silver halide emulsion used in the element, the particular desensitizer used, the ratio of gelatin or other colloid binder to silver halide, other components of the emulsions, and the procedure for preparing the emulsions. All of these factors would be well known to one skilled as a maker of silver halide emulsions. Thus, the amount should be effective to provide for a reduction in visible and UV light sensitivity, but no reduction in sensitivity to X-radiation.

More particularly, the useful amount of desensitizer in the elements is at least 1.5 mg/m<sup>2</sup> on each side of the support, and preferably at least 1.7 mg/m<sup>2</sup>. Generally, the upper limit of such materials is 4 mg/m<sup>2</sup>, and preferably, less than 3 mg/m<sup>2</sup> is used. Mixtures of desensitizers can be used in one or more layers of the element.

The following example is provided for illustrative purposes, and not to be limiting in any manner.

#### MATERIALS AND METHODS FOR EXAMPLES

A radiographic film was prepared having the following layer arrangement and composition:

|                |                                                            |                          |
|----------------|------------------------------------------------------------|--------------------------|
| Overcoat Layer | Gelatin                                                    | 1.35 g/m <sup>2</sup>    |
|                | Dye I*                                                     | 0.48 g/m <sup>2</sup>    |
|                | Dye II**                                                   | 0.16 g/m <sup>2</sup>    |
| Emulsion Layer | AgBr Emulsion (tabular grains 1.3 $\mu$ m by 0.13 $\mu$ m) | 7.56 g Ag/m <sup>2</sup> |
|                | Gelatin                                                    | 4.92 g/m <sup>2</sup>    |
|                | Dye I*                                                     | 0.16 g/m <sup>2</sup>    |
|                | Dye II**                                                   | 0.11 g/m <sup>2</sup>    |
|                | 6-chloro-4-nitrobenzotriazole                              | 2.1 mg/m <sup>2</sup>    |

-continued

|                        |                                                            |                          |
|------------------------|------------------------------------------------------------|--------------------------|
| Support Emulsion Layer | Polyethylene terephthalate                                 |                          |
|                        | AgBr Emulsion (tabular grains 1.3 $\mu$ m by 0.13 $\mu$ m) | 7.56 g Ag/m <sup>2</sup> |
| 5                      | Gelatin                                                    | 4.92 g/m <sup>2</sup>    |
|                        | Dye I*                                                     | 0.16 g/m <sup>2</sup>    |
|                        | Dye II**                                                   | 0.11 g/m <sup>2</sup>    |
| Overcoat Layer         | 6-chloro-4-nitrobenzotriazole                              | 2.1 mg/m <sup>2</sup>    |
|                        | Gelatin                                                    | 1.35 g/m <sup>2</sup>    |
| 10                     | Dye I*                                                     | 0.48 g/m <sup>2</sup>    |
|                        | Dye II**                                                   | 0.16 g/m <sup>2</sup>    |

Dye I\* is bis[1-(4-carboxyphenyl)-3-methyl-2-pyrazolin-5-one-4] monomethineoxonol.  
Dye II\*\* is 4-(4-dimethylaminobenzylidene)-1-(4-carboxyphenyl)-3-methyl-2-pyrazolin-5-one.

15 The following developing and fixing solutions of Table IV were used in the following example. The pH values were adjusted in each solution by addition of sodium hydroxide, but any other suitable base can be used for this purpose.

TABLE IV

| DEVELOPING SOLUTION COMPONENT                       | I (mmol/l) | II (mmol/l) |
|-----------------------------------------------------|------------|-------------|
| Potassium sulfite                                   | 280        | 280 mmol/l  |
| Benzotriazole                                       | 17         | 17          |
| 25 4-Hydroxymethyl-4-methyl-1-phenyl-3-pyrazolidone | 19         | 19          |
| Ascorbic acid                                       | 200        | 200         |
| pH                                                  | 9.0        | 10.5        |
| FIXING SOLUTION COMPONENT                           | A (mmol/l) | B (mmol/l)  |
| Sodium thiocyanate                                  | 0.92       | 0.92        |
| Sodium thiosulfate                                  | 0.79       | 0.79        |
| Sodium sulfite                                      | 0.16       | 0.16        |
| pH                                                  | 10.5       | 4.5         |

#### Example

The radiographic films described above were exposed to roomlight (500 Lux fluorescent lighting) for 60 seconds, then processed using the various processing solutions noted above at room temperature and under roomlight using the following processing protocol:

Development 30 seconds

Fixing 30 seconds

Washing (water) 20 seconds

45 The films were then evaluated for Dmin and Dmax using conventional sensitometry. The results are shown in the following Table V:

TABLE V

| DEVELOPING SOLUTION | FIXING SOLUTION | Dmin | Dmax | COMMENTS                                                                                      |
|---------------------|-----------------|------|------|-----------------------------------------------------------------------------------------------|
| 50 I                | A               | 0.4  | 1.5  | Invention; good differentiation in density                                                    |
|                     | A               | 3.8  | 4.4  | Comparison; extreme fogging from roomlight exposure                                           |
| II                  | B               | 0.5  | 1.0  | Comparison; poor density differentiation; dye insufficiently decolorized due to low fixing pH |
|                     | B               | 3.5  | 3.9  | Comparison; extreme fogging from roomlight exposure                                           |
| 60                  |                 |      |      |                                                                                               |

65 The results clearly indicate the criticality of the fixing solution having a higher pH than the developing solution in order to provide roomlight handleability because of the

## 11

presence of the dye in the element. The dye is then decolorized during fixing.

The invention has been described in detail with particular reference to preferred embodiments thereof, but it will be understood that variations and modifications can be effected within the spirit and scope of the invention.

We claim:

1. A method for providing a black-and-white image comprising:

A) contacting an imagewise exposed photographic silver halide element with an aqueous black-and-white developing composition having a pH of less than 10, and

B) contacting said element with a fixing composition having a pH of from 10 to about 11.5, and comprising a fixing agent at from about 0.8 to about 2.5 mol/l and a sulfite at from about 0.1 to about 0.3 mol/l,

wherein steps A and B require a total of from about 40 to about 120 seconds, and

said element comprising a support having thereon one or more layers, at least one of said layers being a silver halide emulsion layer,

said element further comprising:

in one of said layers, a microcrystalline particulate dye that absorbs electromagnetic radiation in the visible and UV portions of the spectrum and is decolorized during step B, and

in each of said silver halide emulsion layers, a desensitizer that reduces sensitivity of said silver halide to electromagnetic radiation in the visible portion of the spectrum by trapping electrons generated by exposure to said visible electromagnetic radiation.

2. The method of claim 1 wherein said developing composition has a pH of from about 7 to about 9.5.

3. The method of claim 1 wherein said developing composition is free of dihydroxybenzene developing agents, and comprises an auxiliary co-developing agent and a sulfite preservative.

4. The method of claim 1 wherein said fixing composition has a pH of from 10 to about 11.5.

5. The method of claim 1 wherein said fixing composition comprises said fixing agent at from about 0.8 to about 2.5 mol/l, and said sulfite at from about 0.1 to about 0.3 mol/l.

6. The method of claim 1 wherein step A is carried out within from about 20 to about 60 seconds, and step B is carried out within from about 20 to about 60 seconds.

7. The method of claim 1 wherein said photographic element is a radiographic element having a film support and a silver halide emulsion layer on both sides of said support.

8. The method of claim 1 wherein said dye is a nonionic polymethine dye.

9. The method of claim 8 wherein said dye is present in said element in an amount of from about 0.5 to about 2 g/m<sup>2</sup>.

10. The method of claim 1 wherein said desensitizer is an azomethine dye.

11. The method of claim 10 wherein said desensitizer is present in said element in an amount of from about 1.5 to about 4 mg/m<sup>2</sup>.

12. The method of claim 1 wherein said element comprises a silver halide emulsion layer comprising forehardened silver halide tabular grains.

## 12

13. The method of claim 12 wherein said silver halide emulsion layer comprises tabular grains comprising at least 85 mol % silver bromide.

14. The method of claim 1 further comprising washing said element after step B with a wash solution having a pH of 7 or less.

15. The method of claim 14 that is carried out within 90 seconds.

16. A method for providing a black-and-white image comprising:

A) contacting an imagewise exposed radiographic silver halide element with an aqueous black-and-white developing composition having a pH of from about 8 to about 9.5 and is free of dihydroxybenzene developing agents, but comprises an ascorbic acid developing agent, an auxiliary co-developing agent, a sulfite preservative, and an antifoggant,

B) contacting said element with a fixing composition having a pH of from 10.4 to 11, and comprising a fixing agent at from about 1 to about 2.25 mol/l and a sulfite at from about 0.15 to about 0.25 mol/l, and

C) washing said element with a wash solution having a pH of from about 4.5 to about 7,

said steps A and B requiring a total of from about 60 to about 90 seconds, and

said element comprising a film support having on both sides thereof, at least one silver halide emulsion layer comprising forehardened tabular grains comprising at least 97 mol % silver bromide, and an overcoat layer over each emulsion layer,

said element further comprising on each side of said support from about 0.7 to about 1.5 g/m<sup>2</sup> of a nonionic polymethine particulate dye, and from about 1.7 to about 3 mg/m<sup>2</sup> of an azomethine dye desensitizer.

17. The method of claim 16 wherein said particulate dye is located in each of said overcoat layers.

18. The method of claim 16 wherein said desensitizer is located in each of said tabular grain silver halide emulsion layers.

19. The method of claim 16 being carried out for from about 60 to about 120 seconds.

20. The method of claim 16 wherein

said developing composition has a pH of from about 8 to about 9, said ascorbic acid developing agent is D,L-ascorbic acid or a salt thereof, said developing solution sulfite is potassium sulfite, said co-developing agent is 4-hydroxymethyl-4-methyl-1-phenyl-3-pyrazolidone, and said antifoggant is benzotriazole,

said fixing composition has a pH of from about 10.5 to about 10.8, and comprises a combination of sodium thiocyanate and sodium thiosulfate as fixing agents, and said fixing solution sulfite is sodium sulfite, and steps A and B are carried out for from about 15 to about 30 seconds each.